# EUROPEAN PATENT SPECIFICATION

(11) **EP 2 669 900 B1**
(45) Date of publication and mention of the grant of the patent: **29.07.2015**
(21) Application number: 12739337.9
(22) Date of filing: 24.01.2012
(51) Int. Cl.: H01B 3/02, H01B 3/44, H01B 5/08, H01B 7/14, H01B 7/30, D07B 1/14, H01B 1/02, C22C 9/00, C22C 9/02, C22C 21/00, C22C 21/08, C22F 1/04, C22F 1/05, C22F 1/08

(54) **ELECTRICAL CONDUCTOR FOR TRANSPORTING ELECTRICAL ENERGY AND CORRESPONDING PRODUCTION METHOD**
ELEKTRISCHER LEITER FÜR DEN TRANSPORT ELEKTRISCHER ENERGIE UND ENTSPRECHENDES HERSTELLUNGSVERFAHREN
CONDUCTEUR ÉLECTRIQUE POUR LE TRANSPORT D'ÉNERGIE ÉLECTRIQUE ET PROCÉDÉ DE FABRICATION CORRESPONDANT

(30) Priority: 24.01.2011 EP 11151788; 24.11.2011 ES 201131896
(43) Date of publication of application: 04.12.2013
(73) Proprietor: La Farga Lacambra, S.A., 08509 Les Masies de Voltrega (ES)
(72) Inventor: RIERA FONTANA, Lluis, E-08508 Les Masies de Voltregà (ES); FERRER CRUSELLAS, Núria, E-08508 Les Masies de Voltregà (ES); GARCIA ZAMORA, Miquel, E-08508 Les Masies de Voltregà (ES); GUIXÀ ARDERIU, Oriol, E-08508 Les Masies de Voltregà (ES); GARCÍA MARSÁ, Cristina, E-08508 Les Masies de Voltregà (ES); ESPIELL ÁLVAREZ, Ferran, E-08028 Barcelona (ES)
(74) Representative: Isern-Jara, Nuria
(86) International application number: PCT/ES2012/070036
(87) International publication number: WO 2012/101308

(56) References cited:
- EP-A1- 1 418 595
- EP-A1- 2 204 822
- ES-A1- 2 142 747
- ES-A1- 2 159 225
- ES-T3- 2 083 000
- ES-T3- 2 344 408
- JP-A- H0 547 230
- US-A- 3 647 563
- US-A1- 2010 018 745

## Description

### Feld of the Invention

The invention relates to an electrical conductor for the transmission of electrical power, where the conductor has a total cross-sectional area equal to or over 10 mm2 and comprises a plurality of stranded filamentary members. The filamentary members can be, for example, wires of circular cross-section, wires of trapezoidal cross-section, wires of triangular cross-section, as well as other possible sections.

The invention also relates to a process for manufacturing an electrical conductor according to the invention.

The invention also relates to applications of conductors according to the invention, such as for example overhead power lines and submarine cables that comprise a conductor according to the invention.

### State of the Art

In the field of the transmission and distribution of electrical power by means of overhead lines aluminum-steel (ACSR) electrical conductors are well known.

The consumption of electrical power is constantly increasing. This requires, on the one hand, new facilities of increasingly greater capacity and, on the other hand requires the introduction of changes in the present facilities so that they can carry more power

### Summary of the invention

It is an object of the invention to contribute novel solutions to this situation. This purpose is achieved by means of an electrical conductor of the type mentioned hereinabove characterized in that at least one of the filamentary members (and preferably all of them) is made from unannealed microalloyed copper, with a minimum copper content of 98 wt%, or from a unannealed microalloyed aluminum, with a minimum aluminum content of 90 wt%, and has its side surface totally coated with a fluorinated polymer.

The fluorinated polymers are those polymers based on fluorocarbons, with multiple C-F bonds. Within the fluorinated polymer group the following are to be found:
- Polyvinyl fluorides (PVF)
- Polyvinylidene fluorides (PVDF)
- Perfluoroalkoxys (PFA)
- Polytetrafluoroethylene (PTFE)
- Fluorinated ethylene propylene (FEP)
- Ethylene tetrafluoroethylene (ETFE)
- Ethylene chlorotrifluoroethylene (ECTFE)
- Perfluorinated elastomers
- Chlorotrifluoroethylene vinylidene fluoride
- Perfluoropolyether
- Polichlorotrifluoroethylene

In fact, an effect known as "skin effect" occurs in the electrical conductors. In direct current, the current density is similar throughout the conductor, but in alternating current a greater current density is observed on the surface than in the center. This phenomenon is known as skin effect and means that the resistance of a conductor to the flow of alternating current is greater than to the flow of direct current. The skin effect is due to the variation of the magnetic field being greater in the center of the conductor, giving rise to a greater inductive reactance, and, due to this, to a smaller intensity in the center of the conductor and a larger intensity at the periphery. At high frequencies the electrons tend to circulate by the most external zone of the conductor, in corona form, instead of over the entire section, whereby, in fact, the effective cross section over which these electrons circulate is reduced, increasing the resistance of the conductor. In the case of stranded electrical conductors, since the wires (in general, the filamentary members) are in mutual electrical contact, the skin effect is observed as if the stranded electrical conductor were a single conductor of greater cross section. Nevertheless, when at least one filamentary member is coated with a fluorinated polymer, the insulating properties of the fluorinated polymer allow the coated filamentary member to be insulated from the rest, whereby the skin effect affects the filamentary member in a way isolated from the rest. The result is that the overall skin effect is smaller, allowing the electrical resistance of the electrical conductor to be reduced in alternating current.

The improved behavior to the skin effect is thanks to the insulating properties of the fluorinated compound. Furthermore, the fluorinated compounds withstand high temperatures, allowing the conductor to work at high temperatures without the coating becoming degraded.

This combination of advantages makes the conductors according to the invention particularly appropriate for any application related to the transmission of electrical power.

The corona effect is an electrical phenomenon that takes place in electrical conductors and appears as a luminous glow around them. Since the conductors usually have a circular cross section, the glow adopts the form of a corona, whereby the name of the phenomenon.

The corona effect is caused by the ionization of the air surrounding the conductor due to the voltage levels in the line. When the air molecules ionize, they are capable of conducting the electrical current and part of the electrons flowing along the line move on to flow through the air. The intensity of the corona effect, therefore, may be quantified according to the color of the glow, which will be reddish in slight cases and bluish in the more severe ones. The fluorinated polymer coating, specially applied in the outer filamentary members of the conductor, increases by up to 35% the voltage as from which the corona effect takes place (dielectric breakdown voltage), and therefore the power losses caused by the corona effect are reduced.

Additionally, the fluorinated polymer is highly hydrophobic. This is a particularly useful feature since it prevents or reduces the accumulation of ice and/or snow on the electrical conductor, above all if at least all the external filamentary members of the electrical conductor have their side surface totally coated with the fluorinated polymer. Thus, an advantageous application of the conductors according to the invention is the installation thereof in overhead power lines for the transmission of electrical power.

Another additional advantage is derived from the fact that the electrical conductor according to the invention has a smaller elastic modulus, due to the low coefficient of friction of the fluorinated polymer. Thus, conventional electrical conductors (without the coating according to the invention) having an elastic modulus between 30,000 and 40,000 MPa (megapascals), then have an elastic modulus of between 4,000 and 10,000 MPa if the filamentary members are coated according to the invention. As a result of this, the suspended electrical conductor will have a smaller sag. In this sense, it is particularly advantageous for the fluorinated polymer to have a static coefficient of friction comprised between 0.08 and 0.2, and a dynamic coefficient of friction comprised between 0.02 and 0.15.

Another particularly interesting application may be the inclusion of the conductors according to the invention in submarine cables for the transmission of electrical power.

As will be seen hereinafter, the present invention is appropriate for any type of electrical conductor although the preferred applications are for electrical conductors in which the filamentary members are wires of circular cross section and have a diameter of between 0.3 and 5 mm each, with a total diameter of the cord of between 3.5 and 35 mm. The direction of lay of the electrical conductor can be right, left or in alternating rings. Furthermore, it can have wires of various diameters in the same cord, and even wire combinations with other geometries (wires of trapezoidal, triangular cross section, tubes, etc.). It is also advantageous for the electrical conductor to be a conductor stranded with wires of circular, trapezoidal and/or triangular cross section, without a tubular core, which allows solutions with a smaller catenary sag to be obtained.

Preferably the electrical conductor has a plurality of fluorinated polymer coated filamentary members (that is to say with the side surface thereof totally coated with the fluorinated polymer), where said coated filamentary members are distributed in such a way that each of the filamentary members not coated with fluorinated polymer is only in contact with fluorinated polymer coated filamentary members. Indeed, with the non-coated filamentary member being in contact only with coated filamentary members, the non-coated filamentary member is really isolated from the other filamentary members, whereby its behavior relative to the skin effect is as if it were coated.

Preferably the filamentary member is made from microalloyed copper with an annealing temperature of above 250°C. Indeed, these materials have proved to be particularly appropriate for the transmission of electrical power by overhead lines. They combine high electrical properties with good mechanical properties, a good resistance to wear and a low thermal fluence. Furthermore their high annealing temperature allows the application thereto of fluorinated polymers requiring high curing temperatures.

Advantageously the composition of the microalloyed copper comprises the following weight percentages:
- Zn: 0.001 - 0.015
- Pb: 0.005 - 0.050
- Sn: 0.005 - 0.600
- Ni: 0.002 - 0.050
- As: 0.001 - 0.005
- Sb: 0.001 - 0.010
- Ag: 0.002 - 0.012
- Mg < 0.4

Preferably the mechanical strength of the electrical conductor is between 400 and 700 MPa.

In another preferred configuration, the filamentary member is made from microalloyed aluminum with an annealing temperature of above 250°C. The main advantage of this material is its lightness and its high annealing temperature also allows the application thereto of fluorinated polymers requiring high curing temperatures.

Advantageously the composition of the microalloyed aluminum comprises the following weight percentages:
- Ag ≤ 0.020
- As ≤ 0.010
- Fe ≤ 0.800
- Ni ≤ 0.015
- Mg ≤ 0.900
- Pb < 0.020
- Si ≤ 0.900
- Ti ≤ 1.800
- Zr ≤ 0.900
- Zn ≤ 0.020
- Se ≤ 0.010
- Te ≤ 0.010
where the sum of the percentages of these components is at least 0.25 wt% of the total alloy.

Either of the following two compositions of microalloyed aluminum (in wt %) are particularly advantageous
- Mg: 0.60 - 0.90
- Si: 0.55 - 0.85
- Al: rest
and
- Zr: 0.15 - 0.25
- Fe: 0.1 - 0.2
- Zn: 0.01 - 0.015
- Ti: ≤ 0.005
- Al: rest

The fluorinated polymer is preferably polytetrafluoroethylene (PTFE) or a derivative thereof. Additionally to the properties already indicated previously, these compounds are very flexible, chemically inert, resistant to sunlight and have non-stick properties.

It is particularly advantageous for the fluorinated polymer to be a polytetrafluoroethylene reinforced with heat resistant resins that is applied in thicknesses (of dry film) comprised between 10 and 35 microns, and to allow continuous operating temperatures of above 220ºC and intermittent operating temperatures of above 250°C.

The electrical conductors according to the invention have therefore improved properties, which makes them suitable, for example, for replacing the ACSR electrical conductors. They have a greater capacity for the transmission of electrical power (since they allow higher service temperatures to be reached and, in the case of the microalloyed copper, have a lower electrical resistance) but they do not increase the suspended weight, whereby they can be used with the existing structures, with no need to reinforce them. Furthermore, in adverse meteorological conditions they prevent or reduce the accumulation of ice and/or snow, which avoids the fall/breakage of the electrical conductors or of the elements that support them.

The invention also has as object a process for the manufacture of an electrical conductor according to the invention characterized in that it comprises a step of coating at least one of the filamentary members with a fluorinated polymer and later stranding of said electrical conductor. Preferably the coating step includes a step of applying said fluorinated polymer by spraying, dipping or impregnation using rollers, and a step of curing the fluorinated polymer at a temperature of above 200ºC, preferably above 220ºC. Indeed, at these curing temperatures the optimal properties of the fluorinated polymer are obtained, and for that reason it is advantageous for the material of the filamentary members to have an annealing temperature above the curing temperature of the fluorinated polymer.

### Brief description of the Drawings

Other advantages and features of the invention are appraised from the following description, in which, without any limiting nature, preferred embodiments of the invention are disclosed, with reference to the accompanying drawings, in which:
Figs. 1 to 5 show cross sections of electrical conductors according to the invention.

### Detailed Description of Embodiments of the Invention

Figs. 1 to 5 show various alternatives of electrical conductors according to the invention. Those filamentary members that are coated with a fluorinated polymer have been shown with a hatched cross section and those that do not have a fluorinated polymer coating have been shown with a plain cross section. In general, the electrical conductors are made from microalloyed copper according to the previously indicated composition.

Fig. 1 shows an electrical conductor of 19 wires 1. Each wire 1 has a diameter of 2.5 mm and the electrical conductor has a cross section of 95 mm². In this case, all the filamentary members (which are wires 1 of circular cross section) are coated.

Fig. 2 also shows an electrical conductor of 19 wires 1. Each wire 1 has a diameter of 3.5 mm and the electrical conductor has a cross section of 125 mm². In this case, all the wires 1 of the outer ring 3 and the internal wire are coated, whereas those of the intermediate ring 5 are coated alternately. In this way, there is obtained the maximum reduction of the skin effect (since there is no electrical connection between any of the wires 1) and the maximum hydrophobic effect (since all the external surface is coated with the hydrophobic polymer). Nevertheless, it has not been necessary to coat three of the wires 1.

Fig. 3 again shows an electrical conductor of 19 wires 1. In this case, each wire 1 has a diameter of 1.5 mm and the electrical conductor has a cross section of 60 mm². The electrical conductor presents another possible combination of coated and uncoated wires 1 that, for example, could be used in applications in which the hydrophobic effect is not important.

The electrical conductor of Fig. 4 has one wire 1 in the interior and two layers of trapezoidal wires 7. All the filamentary members are coated with a fluorinated polymer.

Fig. 5 shows a possible combination of techniques. On the one hand, the electrical conductor has the filamentary members of the intermediate ring 5 (wires 1 of circular cross section) coated with a fluorinated polymer, whereas the external filamentary members (which are trapezoidal wires 7) are coated only on the part of their side surface that is in contact with the environment. With this geometry a good control of the skin effect is obtained, since intermediate ring 5 effectively insulates the three layers of filamentary members (from the point of view of the skin effect it is not important for the filamentary members that are at the same distance from the center, that is to say, in the same ring, to be in electrical contact with each other), whereas also a good hydrophobicity is obtained. Furthermore, in general, the fact that an electrical conductor has its outer ring 3 formed with trapezoidal wires 7 reduces the accumulation of snow/ice since it has a smoother external surface and without recesses.

### Example 1:

A comparative test was carried out between a 95 mm² microalloyed copper cord with all the wires coated with Xylan 1514 ® (a polymer composed of polytetrafluoroethylene reinforced with heat resistant resins marketed by Whitford Plastics Ltd. It has a static coefficient of friction of 0.15, and a dynamic coefficient of friction of 0.06), and a cord of the same composition and geometry but without using the coating. The installation was 70 meters in length. When the same voltage was applied to both electrical conductors, the following results were obtained:
- with the coated cord, a current intensity of 595 A was reached and a sag of 42 cm
- with the uncoated cord, a current intensity of 555 A was reached and a sag of 62 cm
- in both cases, the conductor temperature reached 120ºC.

Conclusions: with the electrical conductor formed by coated wires 8% more electrical current is transmitted, and the installation has 48% less sag.

### Example 2:

A type LA-180 ACSR cable (180 mm²) can work continuously at a maximum temperature of 85ºC, which corresponds to a maximum intensity of 425 A. An equivalent conductor thereto, with no need to reinforce the structures, is equivalent to the 95 mm² microalloyed copper conductor (object of the present invention). This conductor can operate continuously at up to 150ºC, and under these conditions, if the wires thereof are coated alternately with fluorinated polymer it can transport an intensity of 700 A. That is to say, 65% more electrical power.

### Example 3:

Process of application of the fluorinated polymer:
1. Cleaning of the substrate (degreasing)
2. Spraying. It may also be deposited by a dipping or roller impregnation process.
3. If the fluorinated polymer comes in liquid state, it requires drying: 10 min at from 100 to 175°C
4. Curing: less than 30 minutes at temperatures between 220°C and 275°C

As the curing conditions are at temperatures of above 220°C, if this process is carried out on materials having a lower annealing temperature, their mechanical properties will be affected negatively. Therefore it is particularly advantageous for the conductive material to have an annealing temperature of above the curing temperature. It must be remembered that pure aluminum has an annealing temperature below 120ºC, and the annealing temperature of electrolytic copper (ETP) is below 200ºC.

## Claims

1. An electrical conductor for the transmission of electrical power, where said conductor has a total cross section equal to or more than 10 mm² and comprises a plurality of stranded filamentary members (1, 7), **characterized in that** at least one of said filamentary members (1, 7) is made from unannealed microalloyed copper, with a minimum copper content of 98 wt%, or from unannealed microalloyed aluminum, with a minimum aluminum content of 90 wt%, and has its side surface totally coated with a fluorinated polymer.

2. The electrical conductor according to claim 1, **characterized in that** it is a stranded electrical conductor having wires (1, 7) of circular, trapezoidal and/or triangular cross section, without a tubular core.

3. The electrical conductor according to one of claims 1 or 2, **characterized in that** it is formed by wires (1) of circular cross section having a diameter of between 0.3 mm and 5 mm.

4. The electrical conductor according to anyone of claims 1 to 3, **characterized in that** it has a plurality of filamentary members (1, 7) coated with fluorinated polymer, where said coated filamentary members (1, 7) are distributed in such a way that each of the filamentary members (1, 7) not coated with fluorinated polymer is only in contact with filamentary members (1, 7) coated with fluorinated polymer.

5. The electrical conductor according to anyone of claims 1 to 4, **characterized in that** all the external filamentary members (1, 7) thereof have their side surface totally coated with said fluorinated polymer.

6. The electrical conductor according to anyone of claims 1 to 5, **characterized in that** said microalloyed copper has an annealing temperature higher than the curing temperature of said fluorinated polymer.

7. The electrical conductor according to anyone of claims 1 to 6, **characterized in that** said microalloyed copper has an annealing temperature of above 250ºC.

8. The electrical conductor according to anyone of claims 1 to 7, **characterized in that** the composition of said microalloyed copper comprises the following weight percentages:
- Zn: 0.001 - 0.015
- Pb: 0.005 - 0.050
- Sn: 0.005 - 0.600
- Ni: 0.002 - 0.050
- As: 0.001 - 0.005
- Sb: 0.001 - 0.010
- Ag: 0.002 - 0.012
- Mg < 0.4

9. The electrical conductor according to anyone of claims 1 to 5, **characterized in that** said microalloyed aluminum has an annealing temperature higher than the curing temperature of said fluorinated polymer.

10. The electrical conductor according to anyone of claims 1 to 5 and 9, **characterized in that** said microalloyed aluminum has an annealing temperature of above 250°C.

11. The electrical conductor according to anyone of claims 1 to 5, 9 and 10, **characterized in that** the composition of said microalloyed aluminum comprises the following weight percentages.
- Ag ≤ 0.020
- As ≤ 0.010
- Fe ≤ 0.800
- Ni ≤ 0.015
- Mg ≤ 0.900
- Pb ≤ 0.020
- Si ≤ 0.900
- Ti ≤ 1.800
- Zr ≤ 0.900
- Zn ≤ 0.020
- Se ≤ 0.010
- Te ≤ 0.010
where the sum of the percentages of these components is at least 0.25 wt% of the total alloy.

12. The electrical conductor according to anyone of claims 1 to 5, 9 and 10, **characterized in that** the composition of said microalloyed aluminum comprises the following weight percentages.
- Mg: 0.60 - 0.90
- Si: 0.55 - 0.85
- Al: rest

13. The electrical conductor according to anyone of claims 1 to 5, 9 and 10, **characterized in that** the composition of said microalloyed aluminum comprises the following weight percentages.
- Zr: 0.15 - 0.25
- Fe: 0.1 - 0.2
- Zn: 0.01 - 0.015
- Ti: ≤ 0.005
- Al: rest

14. The electrical conductor according to anyone of claims 1 to 13, **characterized in that** said fluorinated polymer is polytetrafluoroethylene or a derivative thereof.

15. The electrical conductor according to anyone of claims 1 to 14, **characterized in that** said fluorinated polymer is polytetrafluoroethylene with heat resistant resins.

16. The electrical conductor according to anyone of claims 1 to 15, **characterized in that** the thickness of the dry film of said fluorinated polymer is comprised between 10 and 35 microns.

17. The conductor according to anyone of claims 1 to 16, **characterized in that** all the filamentary members (1, 7) thereof are made from microalloyed copper.

18. The conductor according to anyone of claims 1 to 16, **characterized in that** all the filamentary members (1, 7) thereof are made from microalloyed aluminum.

19. A process for the manufacture of an electrical conductor for the transmission of electrical power according to anyone of claims 1 to 18, **characterized in that** it comprises a step of coating at least one of said filamentary members (1, 7) with a fluorinated polymer and subsequent stranding of said electrical conductor.

20. The process according to claim 19, **characterized in that** said coating step includes a step of applying said fluorinated polymer by spraying, dipping or impregnation by means of rollers, and a curing step of said fluorinated polymer at a temperature of above 200ºC, preferably above 220°C.

21. An overhead power line for the transmission of electrical power, **characterized in that** it comprises at least one conductor according to anyone of claims 1 to 18.

22. A submarine cable for the transmission of electrical power, **characterized in that** it comprises at least one conductor according to anyone of claims 1 to 18.

## Patentansprüche

1. Elektrischer Leiter zur Übertragung von elektrischem Strom, wobei der genannte Leiter einen Gesamtquerschnitt von 10 mm² oder mehr aufweist und eine Vielzahl an verlitzten faserartigen Teilen (1, 7) umfasst, **dadurch gekennzeichnet, dass** zumindest eines der genannten faserartigen Teile (1, 7) aus nicht geglühtem mikrolegiertem Kupfer mit einem Mindestkupfergehalt von 98 Gewichts-% oder aus nicht geglühtem mikrolegiertem Aluminium mit einem Mindestaluminiumgehalt von 90 Gewichts-% besteht und seine Seitenfläche vollständig mit einem fluorierten Polymer beschichtet ist.

2. Elektrischer Leiter nach Anspruch 1, **dadurch gekennzeichnet, dass** er ein verlitzter elektrischer Leiter ist, welcher Drähte (1, 7) mit kreisförmigem, trapezförmigem und/oder dreieckigem Querschnitt ohne einen röhrenförmigen Kern aufweist.

3. Elektrischer Leiter nach einem der Ansprüche 1 oder 2, **dadurch gekennzeichnet, dass** er durch Drähte (1) mit kreisförmigem Querschnitt gebildet ist, welche einen Durchmesser zwischen 0,3 und 5 mm haben.

4. Elektrischer Leiter nach einem der Ansprüche 1 bis 3, **dadurch gekennzeichnet, dass** er eine Vielzahl an faserartigen Teilen (1, 7) aufweist, welche mit fluoriertem Polymer beschichtet sind, wobei die genannten beschichteten faserartigen Teile (1, 7) derart verteilt sind, dass jedes der faserartigen Teile (1, 7), welches nicht mit fluoriertem Polymer beschichtet ist, lediglich mit faserartigen Teilen (1, 7) in Kontakt steht, welche mit fluoriertem Polymer beschichtet sind.

5. Elektrischer Leiter nach einem der Ansprüche 1 bis 4, **dadurch gekennzeichnet, dass** die Seitenfläche sämtlicher seiner externen faserartigen Teile (1, 7) vollständig mit dem genannten fluorierten Polymer beschichtet ist.

6. Elektrischer Leiter nach einem der Ansprüche 1 bis 5, **dadurch gekennzeichnet, dass** der genannte mikrolegierte Kupfer eine Glühtemperatur aufweist, welche höher als die Aushärtetemperatur des genannten fluorierten Polymers ist.

7. Elektrischer Leiter nach einem der Ansprüche 1 bis 6, **dadurch gekennzeichnet, dass** das genannte mikrolegierte Kupfer eine Glühtemperatur von über 250 °C aufweist.

8. Elektrischer Leiter nach einem der Ansprüche 1 bis 7, **dadurch gekennzeichnet, dass** die Zusammensetzung des genannten mikrolegierten Kupfers folgende Gewichtsprozente umfasst:
- Zn: 0,001 - 0,015
- Pb: 0,005 - 0,050
- Sn: 0,005 - 0,600
- Ni: 0,002 - 0,050
- As: 0,001 - 0,005
- Sb: 0,001 - 0,010
- Ag: 0,002 - 0,012
- Mg: < 0,4.

9. Elektrischer Leiter nach einem der Ansprüche 1 bis 5, **dadurch gekennzeichnet, dass** das genannte mikrolegierte Aluminium eine Glühtemperatur aufweist, welche höher als die Aushärtetemperatur des genannten fluorierten Polymers ist.

10. Elektrischer Leiter nach einem der Ansprüche 1 bis 5 und 9, **dadurch gekennzeichnet, dass** das genannte mikrolegierte Aluminium eine Glühtemperatur von über 250°C aufweist.

11. Elektrischer Leiter nach einem der Ansprüche 1 bis 5, 9 und 10, **dadurch gekennzeichnet, dass** die Zusammensetzung des genannten mikrolegierten Aluminiums folgende Gewichtsprozente umfasst:
- Ag ≤0,020
- As ≤ 0,010
- Fe ≤ 0,800
- Ni ≤ 0,015
- Mg ≤ 0,900
- Pb ≤ 0,020
- Si ≤ 0,900
- Ti ≤ 1,800
- Zr ≤ 0,900
- Zn ≤ 0,020
- Se ≤ 0,010
- Te ≤ 0,010
wobei die Summe der Prozentanteile dieser Bestandteile zumindest 0,25 Gewichts-% der gesamten Legierung beträgt.

12. Elektrischer Leiter nach einem der Ansprüche 1 bis 5, 9 und 10, **dadurch gekennzeichnet, dass** die Zusammensetzung des genannten mikrolegierten Aluminiums folgende Gewichtsprozente umfasst:
- Mg: 0,60 - 0,90
- Si: 0,55 - 0,85
- Al: Rest.

13. Elektrischer Leiter nach einem der Ansprüche 1 bis 5, 9 und 10, **dadurch gekennzeichnet, dass** die Zusammensetzung des genannten mikrolegierten Aluminiums folgende Gewichtsprozente umfasst:
- Zr: 0,15 - 0,25
- Fe: 0,1 - 0,2
- Zn: 0,01 - 0,015
- Ti: ≤ 0,005
- Al: Rest.

14. Elektrischer Leiter nach einem der Ansprüche 1 bis 13, **dadurch gekennzeichnet, dass** das genannte fluorierte Polymer Polytetrafluorethylen oder ein Derivat davon ist.

15. Elektrischer Leiter nach einem der Ansprüche 1 bis 14, **dadurch gekennzeichnet, dass** das genannte fluorierte Polymer Polytetrafluorethylen mit hitzebeständigen Wachsen ist.

16. Elektrischer Leiter nach einem der Ansprüche 1 bis 15, **dadurch gekennzeichnet, dass** die Dicke des trockenen Films des genannten fluorierten Polymers zwischen 10 und 35 Mikrometer beträgt.

17. Leiter nach einem der Ansprüche 1 bis 16, **dadurch gekennzeichnet, dass** sämtliche faserartigen Teile (1, 7) davon aus mikrolegiertem Kupfer bestehen.

18. Leiter nach einem der Ansprüche 1 bis 16, **dadurch gekennzeichnet, dass** sämtliche faserartigen Teile (1, 7) davon aus mikrolegiertem Aluminium bestehen.

19. Verfahren zur Herstellung eines elektrischen Leiters zur Übertragung von elektrischem Strom nach einem der Ansprüche 1 bis 18, **dadurch gekennzeichnet, dass** es einen Schritt des Beschichtens von zumindest einem der genannten faserartigen Teile (1, 7) mit einem fluorierten Polymer und ein darauffolgendes Verlitzen des genannten elektrischen Leiters umfasst.

20. Verfahren nach Anspruch 19, **dadurch gekennzeichnet, dass** der genannte Beschichtungsschritt einen Schritt des Aufbringens des genannten fluorierten Polymers durch Sprühen, Eintauchen oder Imprägnieren durch Walzen, sowie einen Schritt des Aushärtens des genannten fluorierten Polymers bei einer Temperatur von über 200 °C, vorzugsweise von über 220 °C, beinhaltet.

21. Überlandleitung zur Übertragung von elektrischem Strom, **dadurch gekennzeichnet, dass** sie zumindest einen Leiter nach einem der Ansprüche 1 bis 18 umfasst.

22. Unterseekabel zur Übertragung von elektrischem Strom, **dadurch gekennzeichnet, dass** es zumindest einen Leiter nach einem der Ansprüche 1 bis 18 umfasst.

## Revendications

1. Conducteur électrique pour la transmission d'énergie électrique, dans lequel ledit conducteur a une section transversale totale égale ou supérieure à 10 mm² et comprend une pluralité de membres filamentaires toronnés (1, 7), **caractérisé en ce que** l'un au moins desdits membres filamentaires (1, 7) est réalisé à partir de cuivre microallié non recuit, avec une teneur minimum en cuivre de 98 wt%, ou à partir d'aluminium microallié non recuit, avec une teneur minimum en aluminium de 90 wt%, et a sa surface latérale totalement enrobée de polymère fluoré.

2. Conducteur électrique selon la revendication 1, **caractérisé en ce que** c'est un conducteur électrique toronné ayant des câbles (1, 7) de section transversale circulaire, trapézoïdale et/ou triangulaire, sans coeur tubulaire.

3. Conducteur électrique selon l'une quelconque des revendications 1 ou 2, **caractérisé en ce qu'**il est formé par des câbles (1) de section transversale circulaire ayant un diamètre compris entre 0,3 mm et 5 mm.

4. Conducteur électrique selon l'une quelconque des revendications 1 à 3, **caractérisé en ce qu'**il a une pluralité de membres filamentaires (1, 7) enrobés de polymère fluoré, dans lequel lesdits membres filamentaires enrobés (1, 7) sont répartis de telle sorte que chacun des membres filamentaires (1, 7) non enrobés de polymère fluoré est uniquement en contact avec des membres filamentaires (1, 7) enrobés de polymère fluoré.

5. Conducteur électrique selon l'une quelconque des revendications 1 à 4, **caractérisé en ce que** tous les membres filamentaires externes (1, 7) de celui-ci ont leur surface latérale complètement enrobée dudit polymère fluoré.

6. Conducteur électrique selon l'une quelconque des revendications 1 à 5, **caractérisé en ce que** ledit cuivre microallié a une température de recuit supérieure à la température de durcissement dudit polymère fluoré.

7. Conducteur électrique selon l'une quelconque des revendications 1 à 6, **caractérisé en ce que** ledit cuivre microallié a une température de recuit au-dessus de 250 °C.

8. Conducteur électrique selon l'une quelconque des revendications 1 à 7, **caractérisé en ce que** la composition dudit cuivre microallié comprend les pourcentages de poids suivants :
- Zn : 0,001 - 0,015
- Pb: 0,005 - 0,050
- Sn : 0,005 - 0,600
- Ni : 0,002 - 0,050
- As : 0,001 - 0,005
- Sb: 0,001 - 0,010
- Ag : 0,002 - 0,012
- Mg < 0,4.

9. Conducteur électrique selon l'une quelconque des revendications 1 à 5, **caractérisé en ce que** ledit aluminium microallié a une température de recuit supérieure à la température de durcissement dudit polymère fluoré.

10. Conducteur électrique selon l'une quelconque des revendications 1 à 5 et 9, **caractérisé en ce que** ledit aluminium microallié a une température de recuit au-dessus de 250 °C.

11. Conducteur électrique selon l'une quelconque des revendications 1 à 5, 9 et 10, **caractérisé en ce que** la composition dudit aluminium microallié comprend les pourcentages de poids suivants.
- Ag ≤ 0,020
- As ≤ 0,01 0
- Fe ≤ 0,800
- Ni ≤ 0,015
- Mg ≤ 0,900
- Pb ≤ 0,020
- Si ≤ 0,900
- Ti ≤ 1,800
- Zr ≤ 0,900
- Zn ≤ 0,020
- Se ≤ 0,010
- Te ≤ 0,010
dans lequel la somme des pourcentages de ces composants est au moins de 0,25 wt% de l'alliage total.

12. Conducteur électrique selon l'une quelconque des revendications 1 à 5, 9 et 10, **caractérisé en ce que** la composition dudit aluminium microallié comprend les pourcentages de poids suivants.
- Mg : 0,60 - 0,90
- Si : 0,55 - 0,85
- Al : restes.

13. Conducteur électrique selon l'une quelconque des revendications 1 à 5, 9 et 10, **caractérisé en ce que** la composition dudit aluminium microallié comprend les pourcentages de poids suivants.
- Zr : 0,15 - 0,25
- Fe: 0,1 - 0,2
- Zn : 0,01 - 0,015
- Ti : ≤ 0,005
- Al : restes.

14. Conducteur électrique selon l'une quelconque des revendications 1 à 13, **caractérisé en ce que** ledit polymère fluoré est du polytétrafluoroéthylène ou un dérivé de celui-ci.

15. Conducteur électrique selon l'une quelconque des revendications 1 à 14, **caractérisé en ce que** ledit polymère fluoré est du polytétrafluoroéthylène avec des résines résistantes à la chaleur.

16. Conducteur électrique selon l'une quelconque des revendications 1 à 15, **caractérisé en ce que** l'épaisseur du film sec dudit polymère fluoré est comprise entre 10 et 35 microns.

17. Conducteur selon l'une quelconque des revendications 1 à 16, **caractérisé en ce que** tous les membres filamentaires (1, 7) de celui-ci sont réalisés à partir de cuivre microallié.

18. Conducteur selon l'une quelconque des revendications 1 à 16, **caractérisé en ce que** tous les membres filamentaires (1, 7) de celui-ci sont réalisés à partir d'aluminium microallié.

19. Procédé pour la fabrication d'un conducteur électrique pour la transmission d'énergie électrique selon l'une quelconque des revendications 1 à 18, **caractérisé en ce qu'**il comprend une étape d'enrobage de l'un au moins desdits membres filamentaires (1, 7) avec un polymère fluoré et un taronnage subséquent dudit conducteur électrique.

20. Procédé selon la revendication 19, **caractérisé en ce que** ladite étape d'enrobage comporte une étape d'application dudit polymère fluoré par pulvérisation, trempage ou imprégnation au moyen de rouleaux, et une étape de durcissement dudit polymère fluoré à une température au-dessus de 200 °C, de préférence au-dessus de 220 °C.

21. Ligne à haute tension pour la transmission d'énergie électrique, **caractérisée en ce qu'**elle comprend au moins un conducteur selon l'une quelconque des revendications 1 à 18.

22. Câble sous-marin pour la transmission d'énergie électrique, **caractérisé en ce qu'**il comprend au moins un conducteur selon l'une quelconque des revendications 1 à 18.
